

## UNITED STATES PATENT OFFICE

DWIGHT T. EWING, OF EAST LANSING, MICHIGAN

## CHROMIUM PLATING PROCESS

No Drawing.

Application filed January 3, 1927. Serial No. 158,822.

The invention relates to electrolytes for electrodeposition of chromium and to a process for electroplating chromium in a form suitable for commercial requirements.

5 In my copending application Serial No. 126,094, filed July 30, 1926, I have described a method for rendering a solution of chromic acid suitable for electrodeposition of chromium by the addition of certain compounds of 10 metals having oxidizing and reducing properties and at least two valent states. This application deals primarily with a further development along the same general lines and is concerned chiefly with the addition of certain 15 other compounds to the electrolyte for the purpose of obtaining a better finish on the deposition of chromium and a more easily controlled bath.

In the preferred embodiment of the invention the electrolyte consists of a soluble chromium compound such as chromic acid, which in itself is not suitable for electrodeposition of chromium and the electrolyte is rendered suitable for depositing chromium by the addition of a cerium compound, such for example as cerium oxalate, cerium carbonate, etc. Although chromium may be plated from such solutions the results at times are irregular, due to the formation of a brownish 20 film in spots upon the surface of the chromium. Where such areas are found the deposits of chromium seem to be thinner and under certain conditions the film, upon drying the plated object, is quite adherent and 25 buffing is required for its removal. The formation of some of the film may be prevented to a large extent by washing the objects to be plated in a certain manner, but I have discovered another method to prevent its formation which consists in adding to the electrolyte certain additional substances. While 30 there are a large number of different substances which have the property of preventing the brownish film formation, I have found it most advantageous to use a salt of a metal having a low hydrogen over-voltage. The quantity of this material which should be used can not be well stated in terms of weights and volumes because it is a function of such 35 factors as current density, temperature of

bath, concentration of chromic acid, proportion of cerium oxalate or other compound added to the chromic acid, the anode material and the shape of the object to be plated. Therefore the amount of the film-preventing 55 substance which should be added to the electrolyte can best be found by trial, although it may be stated briefly that the amount used should be that quantity which is just necessary to prevent the formation of the film when the operator is working with a clean piece of work, such as an object of brass, steel or nickel. If substantially more than this amount is added, the efficiency of the plating process is somewhat lowered. As an example 60 of some of the substances which have been found to prevent the formation of the brownish film are the following: hydrofluosilic acid, hydrofluoboric acid, or their soluble salts, sulphites or persulphates. 65

As an example of a specific electrolyte suitable for commercial requirements and the process of preparing the solution, the following formula is given:

Add to a liter of water 200 to 300 grams of 70 commercial chromic acid. When this has dissolved, 10 grams of commercial cerium oxalate is added, with stirring, and dissolved. This solution is now treated with a dilute solution of sodium fluosilicate about 1 gram 75 per 100 cc. solution until upon making a trial under the best current density by plating a brass or nickel object (area about 1 square decimeter) no brown film is formed. The 80 temperature of the bath may be about 20° C. 85

Instead of incorporating the cerium oxalate addition agent in a chromic acid solution it may be used in other chromium-carrying electrolytes where the chromium is in the hexavalent state substantially free from trivalent chromium. For example, under certain conditions good deposits can be obtained 90 from a solution containing per liter of solution 290 grams sodium chromate



and 10 grams cerium oxalate.

While in the above formula I have suggested the use of cerium oxalate as a substance for rendering the chromic acid bath 100

suitable for electroplating, it is to be understood that my invention can also be carried out by adding the film-preventing substance to a chromic acid bath having incorporated therein other compounds of cerium such as 5 the oxides, carbonates, sulphates, etc. and in the broader aspects of the invention the film-preventing compound may be added to any solution of a chromium compound which has incorporated therein a compound of a metal having oxidizing and reducing properties and at least two valent states.

The addition of the sodium fluosilicate or the equivalent substances above enumerated 15 to the electrolyte results in an improved deposit of chromium on the object, this deposit being of uniform thickness, bright and lustrous and free from any brownish film. It is believed that one of the reasons why 20 sodium fluosilicate and other fluosilicates have such a beneficial action on the electrolyte is due to the fact that they are inorganic colloidal substances. It is believed essential that the substance be inorganic in character 25 rather than organic because the presence of chromic acid in the electrolyte introduces such strong oxidizing properties that organic matter present is destroyed.

In carrying out the process of electrodeposition of chromium utilizing the improved electrolyte above described, it has been found very advantageous to accurately determine the amount of current in the working circuit, especially when the bath is being used 35 for objects of different shapes or materials. It is therefore desirable to have an ammeter arranged in the working circuit and by using the ammeter I have discovered a method by which the efficiency of the electroplating 40 process may be increased and the proper current density determined for any particular object which is to be plated. My method consists in placing the object in the electrolyte with a small current flowing in the working 45 circuit and gradually increasing the effective voltage on the bath by rheostats or other suitable means and carefully noting the resulting increase of current flowing through the circuit. It has been found that as the 50 voltage is gradually increased the current also is gradually and uniformly increased until a certain critical point is reached where there is a sudden and appreciable drop in the amperage as indicated by the ammeter. It 55 has been found that when the object is plated with the current corresponding to the critical point or a current just slightly greater than the critical point, a very satisfactory deposit of chromium is obtained and the efficiency of the bath is higher than with other 60 current densities.

It is to be understood that the electroplating process as above described can be carried out on steel, copper, or nickel surfaces which 65 are either polished or unpolished, but if it

is desired to obtain a bright polished chromium surface it is preferable to have a polished under surface on which the deposition takes place to avoid subsequent smoothing of the extremely hard chromium plate.

What I claim as my invention is:

1. An electrolyte for electrodeposition of chromium comprising a solution containing principally chromic acid, together with small amounts of cerium oxalate and sodium hydrosilicate.

2. An electrolyte for electrodeposition of chromium comprising a solution containing principally chromic acid and a relatively small amount of a cerium compound.

3. An electrolyte for electrodeposition of chromium comprising a solution containing principally chromic acid and a relatively small amount of cerium oxalate.

4. An electrolyte for electrodeposition of chromium comprising a solution containing as the principal ingredient chromic acid, a relatively small amount of a cerium compound and a soluble fluosilicate.

5. An electrolyte for electrodeposition of chromium comprising a solution containing having oxidizing and reducing properties relatively small amount of a cerium compound and sodium fluosilicate.

6. An electrolyte for electrodeposition of chromium comprising a solution containing as the principal ingredient a chromium compound having the chromium in the hexavalent state substantially free from trivalent chromium and a serium compound.

In testimony whereof I affix my signature.

DWIGHT T. EWING.

70

80

85

90

100

105

110

115

120

125

130